

## UNITED STATES PATENT OFFICE

2,582,079

COMPOSITION FOR ADDITION TO CAST  
IRON OR STEEL

Jerome Strauss, New York, N. Y., and Daniel Leonard Edlund, Bethel, Pa., assignors to Vanadium Corporation of America, New York, N. Y., a corporation of Delaware

No Drawing. Application September 7, 1950,  
Serial No. 183,662

5 Claims. (Cl. 75—123)

**1**  
This invention relates to a novel composition of matter for the control and improvement of the physical properties of cast iron and for other uses, such as the treatment of steel in the molten state.

Cast iron is a generic term which includes gray irons, white cast irons, chilled cast irons and malleable irons. The properties of these metals depend in part upon chemical factors (principally the percentages of carbon and silicon) and in part upon physical factors, both as influenced by conditions related to the manufacturing methods. This is so because cast iron is essentially the product of a process and the influence of the process details are observed in the qualities of the product. Alloying is employed to alter the properties of some cast irons; also some iron castings both alloyed and not alloyed are subjected to thermal treatments to produce desired results in castings for specific uses. The physical structure (i. e. the nature and distribution of the micro-constituents), and consequently the properties of the metal are influenced not only by these several factors but also by adjusting the maximum temperature attained by the molten iron and the cooling rate both during and after solidification.

Cast iron is sometimes considered unsatisfactory as a material of construction because of its low strength and lack of ductility when compared to steel and certain other engineering alloys. In such a comparison cast iron is usually described as being inherently brittle, especially in the as-cast condition; this brittleness can be reduced only to a very limited extent by heat-treatment, except for long and costly treatments applied to irons in the malleable iron composition range.

The cast iron which is most used commercially for construction applications, however, is gray iron, but this term actually covers a wide range of compositions with corresponding widely varying properties. The composition of gray iron is usually confined within the limits .50 to 2.75% silicon and 2.70 to 3.60% total carbon. Within this range of composition the tensile strength may vary from 15,000 to 60,000 pounds per square inch and occasionally higher.

While a part of the carbon present in gray cast iron may be in the combined form as iron carbide, the greater amount is present in elemental form as graphite. The relative amounts of free carbon and combined carbon, as well as the shape, size and distribution of the particles are dependent upon the remaining chemical com-

**2**  
position of the iron and the influences referred to above, namely, maximum temperature in the liquid state, rate of cooling during and after solidification, and types of heat treatment, if any, applied to a solidified casting.

Elements incidental to the production of cast iron may add or detract from its properties, such as strength, toughness and ductility. Sulphur, for example, is usually kept as low as possible because while it increases the strength of the iron to some degree, it very markedly reduces ductility. Control of sulphur depends, however, on raw materials and process and often it cannot be held to very low values because only high-sulphur raw materials are available, the cost of electric furnace refining may not be permissible and chemical treatment may not be adequate or sufficiently uniform. Phosphorus occasionally strengthens iron but in large amounts renders it quite brittle.

20 Certain elements usually considered as alloying agents have been added to control the structure and properties of cast iron. In some cases the addition of such alloys results in one property being improved to the detriment of another, for example, strength may be improved but the toughness of the iron be reduced unless some adequate form of heat-treatment is provided to retain the toughness. In other cases improvement in strength is accompanied by reduction in the machinability of the iron; in some of these cases heat-treatment, such as annealing, may restore the machinability.

It is known that magnesium added to iron which would otherwise cast gray or nearly so contributes to this iron high strength and some ductility. The ductility has in some cases been found to be increased by an annealing treatment with relatively little sacrifice in this superior strength.

40 However, serious difficulties have beset attempts to make this magnesium practice one that would provide with assurance successive reproduction in continuous manufacturing operations of iron articles of high strength or high strength and good ductility. The boiling point of magnesium being considerably below both the melting temperatures of those metals with which it is preferably combined for making addition agents and below the temperatures at which cast iron is tapped and poured, causes extreme difficulty in controlling the overall recovery of magnesium from raw material to the finished cast iron product.

50 The boiling point of magnesium is about 2030°

F., which results in very high losses due to vaporization of the magnesium when it is added to molten copper and molten nickel to produce such addition agents as 20% magnesium and 80% copper, and 20% magnesium and 80% nickel. Further difficulty is presented when it is attempted to introduce iron into these compositions. Iron is a very desirable carrier metal when magnesium is to be introduced into iron alloys, such as gray cast iron or steel. The introduction of iron into the copper or nickel base alloys mentioned above, however, only increase the already high losses of magnesium during manufacture.

Since the temperature of cast iron flowing from the cupola is normally in the range of 2300 to 2800° F., it is obvious that additional losses will be encountered through vaporization when magnesium alloys are added to iron. When pure metallic magnesium is added to cast iron at such pouring temperatures, its volatilization can be explosive in character. Magnesium continues to vaporize as long as the iron remains molten and the time element combined with the initial violent reaction results in variable losses and properties that vary beyond the limits of satisfactory commercial control. The use of alloy addition agents, such as the 20% magnesium and 80% copper, and 20% magnesium and 80% nickel compositions previously mentioned, does not satisfactorily overcome these difficulties. For example, if the cast iron to which such alloys are added is on the high side of the above temperature range, a violent reaction will occur with high losses of magnesium through volatilization as well as loss of metal and danger to the operators through spattering of the molten cast iron. If, on the other hand, the temperature of the iron is low, incomplete solution may occur, resulting in segregation and in variation in both structure and properties throughout the product.

We have discovered in the course of extended experiments directed toward the development of a commercially satisfactory practice for producing magnesium-containing cast iron of predictable and reproducible properties that certain combinations, preferably in alloy form, of magnesium, silicon, manganese and iron afford an unexpected means of simplification of these problems. Primarily, our discovery consists in a certain critical combination in the proportions of magnesium, silicon, manganese and iron, which substantially increases the recovery of magnesium in manufacture of the addition agent as well as when this agent is added to molten cast iron. This combination of effects results in a substantial cost saving. More significant, however, is the fact that, when using alloys of compositions within the limits of our invention, the desired improvements in the finished cast iron are obtainable more readily and with much greater regularity. While cast iron in which substantially all of the carbon is in the form of spheroids has been produced frequently, it has been difficult to obtain structurally perfect castings under production conditions with a variety of designs, melting equipment, raw materials and other foundry conditions. An infinitely closer approach to perfection can be attained in the use of the alloy herein described. The mechanism of the behavior of this magnesium-silicon-manganese-iron composition within the critical ranges hereinafter set forth has not been fully explained but the results have been obtained with such

regularity both in production of the alloy and in its use with gray cast iron over a substantial amount of production and a large number of different foundries that a distinct advance in the art through its use has been established.

The ranges of composition which have produced the advantages described are 5 to 25% magnesium, 20 to 45% silicon, 2 to 12% manganese, the balance substantially all but not less than 20% or more than 60% iron, except for customary impurities and minor elements, such as carbon, sulphur, phosphorus, etc., which generally do not exceed a total of 4%. Nickel is not included among these minor elements; it is present today in some pig irons and in most iron and steel scrap and hence may be present in these alloys up to about 2% and is not detrimental to the functioning of the alloys. In our compositions, aluminum is a detrimental element. It should be kept below 1% and preferably below 0.6%. Within the ranges of composition already cited, we prefer to restrict the relationship of the several elements so that the ratio of silicon to magnesium is not less than about 1:1 and not greater than about 6:1, and the ratio of magnesium to manganese is not less than 1:1 and not greater than 6:1. Following are four examples of compositions within these critical ranges and possessing the preferred ratio of elements which were manufactured and used successfully:

|                | No. 1    | No. 2    | No. 3    | No. 4    |
|----------------|----------|----------|----------|----------|
| 35             | Per cent | Per cent | Per cent | Per cent |
| Magnesium..... | 22.49    | 13.75    | 6.33     | 18.78    |
| Silicon.....   | 35.65    | 34.42    | 33.42    | 37.98    |
| Manganese..... | 4.36     | 10.50    | 4.51     | 3.64     |
| Iron.....      | Balance  | Balance  | Balance  | Balance  |

40 The definite advantages obtained with an iron content between 20% and 60% are twofold: the iron increases the specific gravity of the alloy, aiding it to penetrate the molten metal, and it raises the melting point, thus slowing down the rate of solution in the molten cast iron, effecting more uniform distribution throughout the mass. In addition to melting too rapidly in the absence of iron, the cost of production becomes excessive if the iron is held below about 20%. If the iron content is permitted to exceed 60%, then the magnesium losses during manufacture of the alloy become excessive and very costly, and the rate of solution of such alloys in molten cast iron is too slow and their effectiveness is greatly impaired.

45 By use of alloys having compositions within the described limits, superior results have been achieved in respect to formation of nodules of graphite in cast iron and reduction of shrinkage of cast iron, over and above what had been previously attained by the best known and most widely used alloy, namely, 80% nickel and 20% magnesium, together with the development of maximum amounts of tensile strength.

50 The amount of alloy added to molten cast iron to be cast into gray iron castings varies with the nature of the iron (as influenced by the raw materials used and the conditions of processing during melting), the maximum temperature attained by the molten iron, the temperature at which the addition is made, the sulphur content of the iron and perhaps other factors. In general, the addition approximates 0.12% to 0.20% of contained magnesium plus an amount of contained magnesium equal to 1½ times the sul-

phur content of the iron. This is not an absolute amount but varies according to the precise composition of the alloy being used as well as the various factors influencing the character of the molten cast iron, as pointed out above, and the method of adding the alloy to the molten iron. It is, however, a good starting point in establishing the practice in a specific foundry while on a particular melting practice so that a limited amount of experimentation varying the addition upward and downward readily establishes the optimum addition required. In general, the amount of alloy added should be such as to leave in the solidified cast iron a total magnesium content of 0.04 to 0.10%, preferably 0.05 to 0.08%.

Another advantage possessed by these alloy addition agents is that of increased recovery of magnesium during both the manufacturing process and during use in the treatment of gray iron. Alloys within these ranges of composition have the peculiar characteristic of being dissolved sufficiently easily in cast iron that they may be effectively used at the lowest customary pouring temperatures which characterize modern commercial foundry practice. On the other hand, solution is sufficiently slow that the alloy and its components will be uniformly distributed throughout the melt and the magnesium will not be lost so rapidly as to prevent it from exerting its influence throughout the entire mass of cast iron. No additional care and no modifications of prior practice are required, the addition of the alloy to iron that would otherwise cast gray, and of low to moderate strength, being the sole requisite. The reason or reasons why these alloys melt at such critical rates so as to be usable at full effectiveness over such a wide range of casting temperatures, but still melt slowly enough so that all ingredients, and particularly the magnesium are distributed uniformly throughout the cast iron have not been clarified but the observations have been sufficiently numerous to be conclusive.

When alloys within composition ranges of the present invention are added to cast iron, increases in strength are secured ranging from about 50% to well over 100%, and the brittle iron becomes ductile, with greatly increased resistance to shock and sudden impact. In improving the mechanical properties to such high degrees the alloys covered by this invention regulate the microstructure of the gray iron so as to produce nodular graphite in the required amount, usually to the extent of complete conversion of the carbon to this form.

The presence of manganese in these alloys gives rise to two outstanding and unpredictable effects. The first is the contribution toward the recovery of magnesium in the preparation of the addition alloys. The second is the part played by manganese as a component of these alloys and their effects upon the cast iron being treated. In this second case the contribution by manganese is different from that which might be expected by one skilled in the art. In the production and usual treatment of cast iron, manganese is a carbide forming element, one of its foremost functions being stabilization of pearlite. Manganese thus increases the tendency of carbon to remain in the combined form. However, as a component of our compositions or alloys the manganese has but mild if any effect on stabilization of carbide and does not interfere with the formation of graphite spheroids.

## Example 1

An outstanding example of the effects of the alloys of this invention upon cast iron was obtained when a particularly weak iron, i. e. low in tensile strength and hardness, was treated with an alloy containing 21.25% magnesium, 34.42% silicon, 4.09% manganese and the balance iron. Analyses of the untreated and treated compositions were as follows:

|                 | T. C. | Mn   | Si   | S     | P     | Mg    |
|-----------------|-------|------|------|-------|-------|-------|
| Untreated.....  | 3.50  | 0.50 | 2.70 | 0.096 | 0.084 |       |
| Mg Treated..... | 2.73  | 0.53 | 3.31 | 0.010 | 0.085 | 0.086 |

The tensile strength and hardness of two bars each of treated and untreated portions of the melt are given below:

|                    | Tensile Strength, p. s. i. | Brinell Hardness |
|--------------------|----------------------------|------------------|
| Untreated.....     | 14,400<br>14,200           | 143<br>111       |
| 25 Mg Treated..... | 77,600<br>89,750           | 255<br>255       |

## Example 2

30 An addition alloy according to the invention and containing 21% magnesium, 34% silicon, 4% manganese and the balance iron was added to a gray iron containing—

|                      | Per cent |
|----------------------|----------|
| 35 Total carbon..... | 3.39     |
| Silicon.....         | 2.27     |
| Manganese.....       | .26      |
| Phosphorus.....      | .024     |
| Sulphur.....         | .01      |

40 An amount of the addition alloy was used to calculate to an addition of .75% magnesium based on the weight of the iron to which it was added.

The physical properties of the treated cast iron were:

|                          |                  |        |
|--------------------------|------------------|--------|
| Tensile strength.....    | lbs. per sq. in. | 62,400 |
| Yield strength.....      | lbs. per sq. in. | 36,300 |
| Elongation.....          | per cent         | 10     |
| Reduction of area.....   | do               | 7.1    |
| 50 Brinell hardness..... |                  | 163    |

## Example 3

55 The addition alloy used in this example contained 24.30% magnesium, 37.79% silicon and 4.06% manganese, the balance being iron. Various quantities of this addition alloy were added to an electric furnace iron having the analysis:

|                      | Per cent |
|----------------------|----------|
| 60 Total carbon..... | 3.73     |
| Silicon.....         | 2.61     |
| Sulphur.....         | .04      |
| Phosphorus.....      | .15      |
| Manganese.....       | .86      |

65 In all cases where the addition of the alloy exceeded 1.50%, the iron was practically all nodular. Tensile tests showed results ranging from 61,450 to 77,100 pounds per square inch. In each case the sulphur was reduced to practically .01%.

70 Methods of sampling and analysis currently in use show after the addition of the alloys of this invention that the carbon content and the sulphur content of the untreated irons have been reduced by the treatment. The reduction in

the sulphur content is no doubt due to the combination of magnesium with at least part of the sulphur and its removal as a slag or a slag forming constituent. The reason for the change in the carbon content is not so obvious and it may be that the change is apparent rather than real due to the difference in the form and the distribution of the carbon and creating a necessity for different methods of sampling and analysis than those commonly in use. Completely satisfactory procedures have not yet been devised or discovered.

It has heretofore been an absolute requirement in the production of cast iron having all or nearly all of its carbon in the form of spheroids that there be added following the addition of the magnesium alloy a second addition rich in silicon, such as ferrosilicon, the amount in most cases being substantial. In the use of the alloys of this invention such final addition of ferrosilicon is not a necessity and may be dispensed with in many cases. The amount of silicon represented by the addition of the alloys according to our invention is very much less than that which would be added according to prior art methods subsequent to the incorporation of the magnesium alloy. Even in those instances where a final addition of silicon-rich alloy is made, the total silicon content represented by this addition plus the silicon content added by means of the magnesium-silicon-manganese-iron alloy is distinctly less than the silicon added as a late ferrosilicon addition according to prior art methods. When the late ferrosilicon addition is actually employed in conjunction with the alloys of this invention, the maximum amount of ferrite in the microstructure may be attained with a minimum silicon addition, leaving not more than a very small amount of pearlitic structure in the matrix and through this means advantage in respect of machinability and reduction in the wear on tools used for machining will result. Production of an iron with minimum pearlite also results in maximum ductility of the iron composition.

While fairly satisfactory results can be obtained in some instances in the treatment of cast iron with compositions of matter within the ranges previously specified, not in the form of alloys but in the form of mechanical mixtures, much better results are obtained by the use of these compositions in alloy form.

Alloys of this invention have also been added to molten steel for lowering the sulphur content of the steel. For example, steels have had their

sulphur content decreased from about .030 to about .020% by the use of these alloys.

The invention is not limited to the preferred embodiment but may be otherwise embodied or practiced within the scope of the following claims.

We claim:

1. A composition of matter for addition to iron or steel, said composition comprising about 5 to 25% magnesium, about 20 to 45% silicon and about 2 to 12% manganese, the balance being substantially all iron, the iron being in an amount between about 20 and 60%.

15 2. An alloy for addition to iron or steel, said alloy comprising about 5 to 25% magnesium, about 20 to 45% silicon and about 2 to 12% manganese, the balance being substantially all iron, the iron being in an amount between about 20 and 60%.

20 3. A composition of matter for addition to iron or steel, said composition comprising about 5 to 25% magnesium, about 20 to 45% silicon and about 2 to 12% manganese, the ratio of silicon to magnesium being between about 1:1 and 6:1, the balance being substantially all iron, the iron being in an amount between about 20 and 60%.

25 4. A composition of matter for addition to iron or steel, said composition comprising about 5 to 25% magnesium, about 20 to 45% silicon and about 2 to 12% manganese, the ratio of magnesium to manganese being between about 1:1 and 6:1, the balance being substantially all iron, the iron being in an amount between about 20 and 60%.

30 5. A composition of matter for addition to iron or steel, said composition comprising about 5 to 25% magnesium, about 20 to 45% silicon and about 2 to 12% manganese, the ratio of silicon to magnesium being between about 1:1 and 6:1, the ratio of magnesium to manganese being between about 1:1 and 6:1, the balance being substantially all iron, the iron being in an amount between about 20 and 60%.

35 6. A composition of matter for addition to iron or steel, said composition comprising about 5 to 25% magnesium, about 20 to 45% silicon and about 2 to 12% manganese, the ratio of magnesium to manganese being between about 1:1 and 6:1, the ratio of magnesium to manganese being between about 1:1 and 6:1, the balance being substantially all iron, the iron being in an amount between about 20 and 60%.

40 7. A composition of matter for addition to iron or steel, said composition comprising about 5 to 25% magnesium, about 20 to 45% silicon and about 2 to 12% manganese, the ratio of magnesium to manganese being between about 1:1 and 6:1, the ratio of magnesium to manganese being between about 1:1 and 6:1, the balance being substantially all iron, the iron being in an amount between about 20 and 60%.

JEROME STRAUSS.

DANIEL LEONARD EDLUND.

#### REFERENCES CITED

The following references are of record in the file of this patent:

#### UNITED STATES PATENTS

| Number       | Name          | Date          |
|--------------|---------------|---------------|
| 1,322,158    | Becket        | Nov. 18, 1919 |
| 1,461,643    | Becket        | July 10, 1923 |
| 55 2,485,760 | Millis et al. | Oct. 25, 1949 |